

R. SEIFFERT.

PROCESS OF OBTAINING METALLIC OXIDS.

APPLICATION FILED DEC. 21, 1905.

902,260.

Patented Oct. 27, 1908.



Witnesses

J. M. Fowler Jr.  
Ruth J. Mitchell

Inventor:

Richard Seiffert,  
By Nixon, Fenwick, Fenwick  
Attorneys.

# UNITED STATES PATENT OFFICE.

RICHARD SEIFFERT, OF BOBREK, GERMANY.

## PROCESS OF OBTAINING METALLIC OXIDS.

No. 902,260.

Specification of Letters Patent.

Patented Oct. 27, 1908.

Application filed December 21, 1905. Serial No. 292,798.

*To all whom it may concern:*

Be it known that I, RICHARD SEIFFERT, engineer, a subject of the German Emperor, residing at Bobrek, Silesia, Germany, have invented certain new and useful Improvements in Processes of Obtaining Metallic Oxids; and I do hereby declare the following to be a full, clear, and exact description of the invention, such as will enable others skilled in the art to which it appertains to make and use the same.

This invention relates to a process for extracting zinc and other metal in a volatile oxidized form, from ore and metallurgical products containing the same. In this process the material to be treated to which the necessary fuel is added, if it does not contain sufficient quantity of combustible substances, such as coal, sulfur, etc., is subjected to the action of an air current which is forced through the mass from below in such manner that the whole charge from top to bottom is brought to the temperature required for volatilizing the zinc and the other volatile ingredients, the said temperature being bright red to white heat. It is essential in this process that the temperature of volatilization should be obtained in the whole charge as uniformly and as simultaneously as possible, and maintained until the volatile ingredients have been completely expelled from all the parts of the charge, and the residue sufficiently deprived of the metals to be extracted.

The drawing illustrates a device which has proved extremely useful for the practical carrying out of the process. The goods are introduced into a cast iron receiver A tapering downwards, the bottom portion of which, serving for introducing blast into the charge, is covered with a perforated plate S. At the commencement of the blowing, incandescent fuel is placed on the perforated plate, and the blast started. Thereupon the receiver is filled with the material to be treated. If the material be introduced in wet state, the pressure of the blast is at first increased in a very gradual manner, so that the material is in this way dried and loosened and made porous by the escaping gases and steam. This stage of the process can be done away with, if the material is supplied to the receiver in dry state. After the material has been sufficiently heated and become permeable to the blast, it is possible, by in-

creasing the pressure of the blast, to bring the whole charge, from the bottom up to the top, in a very short time, to the temperature required for volatilizing zinc. The zinc is thus reduced by the carbon, the zinc fumes, owing to the strong supply of oxygen, burn as soon as they are generated, and the zinc oxide produced is discharged with the gas current into the condensing pipe. Under the influence of the high pressure blast the combustion spreads almost instantaneously throughout the whole mass of the charge. The beginning of this stage can be easily recognized by the sudden flare up and generation of dense smoke. The bringing about of this thermic action in the mass, which communicates almost simultaneously to the whole charge, strong heat being developed at the same time, and the maintaining of the volatilization temperature with the continuous blowing-in of compressed air, are the necessary conditions for the success of the process, more particularly for obtaining high percentage of the required metal oxids.

The inventor has made the observation, in experiments in which he treated masses 1-1½ meters deep, that when the volatilization temperature does not take place as uniformly and as simultaneously as possible in the whole mass, a considerable portion of the zinc oxide produced, becomes condensed in the upper cooler layers of the charge, or a considerable portion of the zinc is altogether unable to escape from the charge. When, on the other hand, the depth of the charge is considerably smaller, apart from the smaller output, the consumption of blast is considerably larger and sometimes considerable losses are experienced owing to the blowing about of the material, the effect sometimes being that the metal oxids obtained are very dirty. As has been proved by experiments, these drawbacks can be obviated with a sufficiently deep charge of the material with the simultaneous use of a correspondingly strong blast pressure, by bringing about the above described "thermic mass action".

In the above case the upper layers of the charge are not enriched by the condensation of the fumes generated. The fumes released in very concentrated form, escape, on the contrary, without any decrease from the surface of the charge and pass through the chimney H into the condensation pipe L.

It has been besides found specially useful,

more particularly when using charges of great depth, and a correspondingly high receiver, to put into the condensation pipe an exhauster or the like, by the suction of which 5 the escape of the fumes, already considerably assisted by the above mentioned method of working, can be still further accelerated.

Apart from the fact that premature condensation of the fumes generated is avoided, 10 it is of essential importance for obtaining high efficiency as regards extraction of metal, that the generation of metal fumes at this stage of the process should take place as quickly and as intensely as possible, for as 15 fritting of the contents of the receiver which takes place during continuous blowing, stops, of course, the unimpeded passage of the blast, and therefore the escape of the fumes generated and their generation. In 20 order therefore to avoid loss of metal, it is necessary in this process that, as far as possible, all the zinc should be expelled before the fritting begins.

When material is being treated which 25 melts easily, it is preferable to bring about the slagging of the charge which, in the above described process must be kept back as much as possible, by forced blowing, immediately after the main generating period, and 30 to continue to blow through the completely liquefied charge with constant increase of the pressure of the blast, until the last traces of the zinc are expelled from the charge melted.

After the blowing process is completed, 35 the receiver A which, as will be seen from the drawing, is arranged so that it can be moved and tipped on a frame, is brought under the chimney and emptied. If the slag at the temperature obtained contains sufficient quantity of non-volatile metals, such as 40 copper, then of course such metals can also be extracted therefrom.

The invention is, of course, not limited to the use of the construction of the blowing 45 apparatus, shown in the drawing. It has been, for instance, found, in experiments made with different materials, that a greater or smaller tapering of the receiver is preferable according to the quality of the material treated. As the volume of the charge 50 considerably decreases during the blowing, as has been proved by experiments, the receiver A can be extended upwards by means of a removable attachment, say, of a cylindrical shape, in order to obtain, at the beginning of the blowing, the greatest possible height of charge.

In view of the exceedingly high temperature in the converter during the blowing, the 60 provision has been made, as shown in the drawing, for cooling the iron walls of the receiver by spraying it by means of a circular rose R. Instead of a converter, could be used a suitably arranged shaft furnace.

65 The process is not limited to purely oxid

ores and smelting products; it can advantageously be applied for blowing ore containing sulfur.

When ore containing sulfur is to be treated for the purpose of extracting from it 70 oxid of zinc, it is advisable to add to it as much lime, dolomite or lime stone in finely divided shape, as is necessary in order that all the  $SO_2$  may combine with the stronger bases,  $CaO, MgO$ , but if it be desired to obtain 75 in the end sulfate of zinc ( $ZnSO_4$ ), then atomized water is introduced into the condensation pipe behind the blowing apparatus, the sulfurous acid being converted with the oxid of zinc into sulfate of zinc. 80 The mixing of the ore with the above mentioned compounds of alkaline earths, in the case of ores, the gangue of which forms a slag which melts too easily, acts at the same time, during the first stage of the process, so 85 as to slightly stiffen the ore and delay the beginning of the slagging.

When it is desired to treat ore which gives a great deal of dust, it is advisable to add to the mixture of ore and coals finely 90 ground lime, dolomite or other suitable binding substance, and the mixture formed into lumps or pieces of any desired shape by any approved means as by the employment of an ordinary briquetting machine. 95

This process has most important advantages, in technical and economical respect, over the well known processes for extracting zinc, for it enables poor ore and waste products, slime residue and the like, to be 100 profitably treated, even where all hitherto known processes have proved inefficient. In many places there are huge heaps of poor galmei which, in view of the present state of the technical science, have been considered as useless. This material can be profitably treated in accordance with this process, as it enables the whole of zinc, up to the last traces, to be expelled and extracted with very cheap machinery and at low working 110 expenses.

#### Claims.

1. The process for extracting zinc and other metals in a volatile oxidized form, 115 from ores and metallurgical products containing the same, consisting in first forcing a blast at low pressure through the ore or smelting product containing the necessary fuel and introduced into a suitable receiver, after the combustion has been started, for 120 the purpose of drying the material and making it porous, and then in increasing the pressure of the blast in such manner, that the temperature, required for the reduction or volatilization of the metals to be expelled, 125 is attained shortly after the starting of the blowing and is communicated almost simultaneously throughout the entire charge, and in continuing the blowing and maintaining the high temperature until the 130

volatile metals to be extracted have been expelled.

2. The process for extracting zinc and other metals in a volatile, oxidized form, from ores and metallurgical products containing the same, consisting in mixing the ore or the smelting products containing the necessary fuel with a suitable binding material, in forming it into lumps or pieces of any desired shape, in forcing through the goods thus prepared and introduced into a suitable receiver, after the starting of the combustion, first a blast of a weak pressure, for the purpose of drying the material and making it porous, then in increasing the pressure of the blast in such manner that the temperature required for the reduction and volatilization of the metals to be expelled, is obtained, shortly after the starting of the blast, throughout the whole depth of the charge, and in continuing the blowing until the volatile metals to be extracted have been expelled.

3. The process for extracting zinc and other metals in volatile oxidized form, from ores and metallurgical products containing the same, consisting in blowing, after the starting of combustion, through the ore or smelting product containing the necessary fuel and introduced into a suitable receiver, a blast of such pressure that the temperature required for the reduction and volatilization of the metals to be expelled is obtained throughout the whole depth of the charge shortly after the starting of the blowing, and in maintaining this temperature by suitable regulation of the pressure of the blast, until

the greater portion of the zinc to be extracted has been obtained, and then by accelerating the blowing in converting the contents of the receiver into liquid state and in blowing with the increased pressure through the molten mass until the zinc has been completely expelled.

4. The process for extracting zinc and other metals in volatile, oxidized form, from ores and metallurgical products containing the same, consisting in blowing through the ore or smelting product containing the necessary fuel, and brought into a suitable receiver, immediately after starting the combustion, a blast of such pressure that the temperature required for the reduction and volatilization of the metals to be extracted is obtained throughout the whole depth of the charge shortly after the starting of the blast, in maintaining the said temperature by suitable regulation of the pressure of the blast until the greater portion of the zinc to be extracted has been expelled, and simultaneously in assisting and accelerating the generation of the metal fumes and their escape from the charge, by suction over the surface of the charge, then in liquefying the contents of the receiver by accelerating the blowing and in continuing the blowing through the liquid mass with an increased pressure until the zinc has been completely expelled.

In testimony whereof, I affix my signature, in presence of two witnesses.

RICHARD SEIFFERT.

Witnesses:

A. N. MAN,  
N. M. WITZ.